

3,183,125  
PROTECTIVE TREATMENT FOR Mg AND  
Mg-BASED ALLOYS

Carl Kenneth Bjork, Midland, Mich., assignor to The Dow Chemical Company, Midland, Mich., a corporation of Delaware  
No Drawing. Filed Mar. 2, 1961, Ser. No. 92,760  
4 Claims. (Cl. 148—6.2)

The invention relates to a method of applying a protective coating to magnesium and magnesium-base alloys and more particularly relates to an improvement in the method of treating particulate magnesium or magnesium-base alloys with an aqueous alkali metal dichromate solution.

For the purposes of the specification and claims magnesium and magnesium-base alloys containing at least 70 percent by weight of magnesium are hereinafter referred to as magnesium metal.

Particulate magnesium metal, during storage as the powder or pellets, tends to react with atmospheric moisture and oxygen and thereby acquires an oxide coating. The coating tends to make the metal less effective in subsequent use in incendiary or explosive compositions and the like. Also, on compounding and then storing such compositions, the metal may become less reactive, or the metal may react with components in the composition whereby the metal is largely consumed before use.

Prior attempts have accordingly been made to provide a protective coating for particulate magnesium metal which does not markedly decrease the reactivity of the metal during rapid combustion or explosive reactions. Heretofore, one of the best ways of protecting particulate magnesium metal has been to form a coating on the particles by subjecting the particulate metal to boiling aqueous dichromate solution for a brief period such as 5-15 minutes whereby a thin protective dichromate conversion coating is formed on the surface of substantially all the particles or pellets. The dichromate coating, perhaps because of its bound oxygen content, has not greatly decreased the reactivity of the metal while providing protection from moisture.

It has now been found that the corrosion resistance of dichromate treated particulate magnesium metal may be further greatly improved, without substantially adversely affecting the reactivity of the metal to rapid combustion or explosive reaction, by the application, to the dichromate treated metal, of a hydrophilic-hydrophobic surface active material having sufficient affinity for the dichromated surface of the metal whereby the surface is made water repellent.

Any magnesium metal may be treated according to the process of the invention, e.g., magnesium, and the magnesium-base alloys having the ASTM or ASTM type designations AZ31A, AZ31B, HK31, ZK60, HM21, ZH11, ZE10A, and the like. Particulate metal having particle sizes up to 0.1 inch diameter or more are advantageously treated according to the invention.

Surface active materials which may be employed are those which are capable of depositing an adherent water repellent covering or layer over the dichromate coating on the magnesium particles. The requisite combination of properties whereby a material is adherent to a chromated magnesium surface, yet is water repellent is found in a hydrophobic, water dispersible, oxygen-containing, surface active compound containing an uninterrupted carbon to carbon chain having from 8 to 26 carbon atoms and a carbon oxygen polar group linkage having sufficient polarity to maintain an affinity for a chromated surface of magnesium.

A surface active material is defined as a material which

lowers the surface tension of water when dispersed therein.

Water repellancy is obtained by having a film of the surface active material substantially covering the individual chromated particles in such a way as to present a hydrophobic surface to the environment of each particle. The water repellancy should be sufficient that the particulate chromated metal particles are not readily wetted by an aqueous solution during at least 15 minutes immersion therein.

Water-dispersable surface active materials includes those that are readily mechanically emulsified in water as well as those that are water soluble.

An uninterrupted carbon to carbon chain containing from 8 to 26 carbon atoms is a sequence of 8 to 26 carbon atoms connected in a series unbroken by intervening non-carbon atoms such as oxygen or nitrogen. The bonding in the sequence may include olefinic bonds, as in the decylenic or linolenic groups, as well as single, or saturated, bonds, as in the lauric or stearic groups.

A carbon oxygen polar group linkage is one having a carbon to oxygen bond, and a substituent atom or group on the oxygen or the carbon whereby the polar group exhibits an asymmetrical displacement of charges, or a dipole effect within the group. The charge separation or the dipole effect must provide sufficient polarity to provide an affinity for the highly ionic chromated surface of the metal so that the polar group is closely held thereto. Under these conditions water, or aqueous solution, does not readily break the bond between the surface active material and the chromated surface. The carbon oxygen polar group linkages include:



Groups of compounds which exhibit the desired combination of properties have a long carbon chain group, as indicated above, to impart hydrophobic character and at least one of carboxy, amino, amido or polyhydroxy groups to impart hydrophylic character. Specific examples of groups of compounds are: alkali metal salts of long chain saturated and unsaturated fatty acids having about 8 to 26 carbon atoms, ethylene oxide condensates of fatty acid amides, amine fatty acid condensates, and alkylphenoxy polyalkoxyalcohols.

For ease of application of the surface active material it is preferred that the material be water dispersable. The material can then be conveniently admixed with, or otherwise incorporated in, the wash water used in the process of dichromate treating the particulate magnesium, though the surface active material may be applied to the particulate magnesium, if desired, as a solution or dispersion in an organic solvent, e.g., ethanol.

In providing chromated particulate magnesium metal, a ground or atomized form of particulate magnesium metal is treated with hot aqueous alkali metal dichromate solution, as well understood in the art, e.g., by treating the metal with from about 5 to 20 cc. of a 10 to 20 percent by weight dichromate solution per gram of metal at about the boiling temperature of the dichromate solution. The metal is usually poured into the hot dichromate solution and the mixture is stirred occasionally during a 10 or 15 minute period. Then the metal is separated from the aqueous solution as by suction filtration.

In carrying out the process of the invention, the dichromate treated metal is washed with an aqueous solution of water and 0.05 to 0.5 percent by weight or more, of a surface active agent of the type defined hereinabove. If the dichromate treated metal has been separated from the dichromate solution by filtration, it is convenient to wash the metal on the filter. About 5 to 10 cc. of the

## 3.

solution of surface active agent per gram of metal provides an adequate treatment.

After the wash solution has filtered or otherwise drained away from the metal, the metal is dried. Air drying may be employed if desired, but oven drying, as at 105-115° C., is to be preferred as quicker and more positive in assuring spreading of the surface active material over the surface of the particle and in enhancing the adherence of the surface active material to the particulate metal.

The beneficial effect of the surface active agent is not entirely understood but it is believed that it is deposited on the dichromated metal as a water repellent layer which seals the pores of the original coating (formed during dichromate treatment) and reduces the wettability of the particulated metal.

## Examples

The following examples serve only to illustrate the advantageous results obtained on following the practice of the invention and the scope of the invention is not to be considered limited thereby.

Portions of ground magnesium powder passing a No. 325 sieve (U. S. Sieve Series), weighing 5 grams, were each placed in a 50 cc. quantity of boiling aqueous sodium dichromate solution (15 grams  $Na_2Cr_2O_7 \cdot 2H_2O$ /100 cc.  $H_2O$ ) for ten minutes. Each dichromated portion was separated from the dichromate solution by suction filtration and washed with a dilute aqueous solution of a water soluble surface active agent, and oven dried at 105- 30 115° C.

By way of comparison, an additional 5 gram portion of ground magnesium powder passing a No. 325 sieve was similarly treated with boiling dichromate solution, separated from the dichromate solution, washed with distilled water, and oven dried.

Each of the dichromate treated portions, including the comparison portion, was tested to determine the relative resistance of the treated powder to corrosive attack by each of 10 percent by weight and 15 percent by weight aqueous perchloric acid solutions. The extent of reaction, i.e., corrosion, of each portion was determined manometrically as follows:

Treated magnesium powder ( $0.2500 \pm 0.0007$  gram) was accurately weighed into a plastic boat. 50 cc. of perchloric acid solution were pipetted into a 500 cc. Erlenmeyer flask. The boat was carefully inserted in the flask so that it floated on the surface of the acid solution and the powder did not contact the acid solution. The flask was closed by a stopper having tubing extending

5

therethrough. The tubing was connected to an open end mercury filled manometer. The flask was shaken causing the boat to tip and bring the magnesium powder into contact with the acid solution. The flask was then immersed in a constant temperature bath maintained at 25° C. The increase in manometric pressure was read after a 15 minute interval. The results of this test and the surface active agents employed are listed in the table.

In a manner similar to that described in the foregoing examples the following surface active compounds or mixtures thereof are found to adhere to dichromate treated particulate magnesium and to impart water repellency thereto:

| Tradename:     | Type of compound                                                                         |
|----------------|------------------------------------------------------------------------------------------|
| Myrj 53        | Polyoxyethylene stearate.                                                                |
| Tween 20       | Polyoxyethylene sorbitan monolaurate.                                                    |
| Brij 35        | Polyoxyethylene lauryl ether.                                                            |
| Renex 20       | Polyoxyethylene ester of mixed fatty and rosin acids.                                    |
| Sipex TEA      | Triethanolamine salt of lauryl alcohol sulfate.                                          |
| Alamine 204    | Secondary fatty amines.                                                                  |
| Amine S        | Alkylated heterocyclic tertiary amine.                                                   |
| Avasol 114     | Fatty acid derivative.                                                                   |
| Cathol         | Fatty amido diamine.                                                                     |
| Ceranine HC    | Fatty amide derivative.                                                                  |
| Ethomeen C/20  | Tertiary amines; ethylene oxide condensation products of the primary fatty amines.       |
| Ethomeen T/15  | Do.                                                                                      |
| Ethomeen T/25  | Do.                                                                                      |
| Ethomeen 18/15 | Do.                                                                                      |
| Ethomid C/15   | Ethylene oxide condensates of fatty acid amides.                                         |
| Ethomid RO/15  | Do.                                                                                      |
| Eureka E-2     | Cationic derivative of a fatty acid diamine condensate.                                  |
| Igepal CA-630  | Octyl phenoxy poly(ethyleneoxy)ethanol.                                                  |
| Igepal CA-730  | Do.                                                                                      |
| Igepal CA-210  | Nonyl phenoxy poly(ethyleneoxy)ethanol.                                                  |
| Janusol        | Mixture of lauryl and myristyl esters containing both primary amino and sulfated groups. |
| Liquex 11      | Fatty acid alkanolamide.                                                                 |

| Sample No.   | Surface active material |                                                   | Extent of corrosion in 15 minutes                  |                                             | Remarks                                                           |
|--------------|-------------------------|---------------------------------------------------|----------------------------------------------------|---------------------------------------------|-------------------------------------------------------------------|
|              | Identity                | Concentration in wash solution, percent by weight | Aqueous $NH_4ClO_4$ , 10%; pressure change, mm. Hg | Concentration, 15%; pressure change, mm. Hg |                                                                   |
| 1            | Intracol OA, C.S.       | 0.5                                               | 0                                                  | 0                                           | Powder wetted very little.                                        |
| 2            | do.                     | 0.25                                              | 5                                                  | 0                                           | Powder wetted slightly by 10% soln., very little by 15% soln.     |
| 3            | do.                     | 0.05                                              | 8                                                  | 12                                          | Powder wetted somewhat.                                           |
| 4            | Aerosol C-61, C.S.      | 0.50                                              | 0                                                  | 0                                           | Powder wetted very little.                                        |
| 5            | Arquad S, C.S.          | 0.50                                              | 15                                                 | 0                                           | Powder wetted somewhat.                                           |
| 6            | Sodium stearate         | 0.25                                              | 0                                                  | 9                                           | Powder wetted very little by 10% soln., somewhat by 15% soln.     |
| 7            | do.                     | 0.10                                              | 3                                                  | 0                                           | Powder wetted very little.                                        |
| 8            | do.                     | 0.05                                              | 2                                                  | 22                                          | Powder wetted very little by 10% soln., some wetting by 15% soln. |
| Comparison A | None                    | 1 None                                            | 26                                                 | (2)                                         | Chromated powder readily wetted by soln.                          |
| Comparison B | do.                     | No wash                                           | (2)                                                | 54                                          | Plain magnesium powder reacted vigorously with acid soln.         |

<sup>1</sup> Distilled water.

<sup>2</sup> Rapid pressure build up too large to measure in apparatus within 1-2 minutes.

Intracol OA, C.S.=Intracol OA cationic surfactant, an acid salt of a long chain fatty acid amide having multiple amine groups on chain.

Aerosol C-61, C.S.=Aerosol C-16 cationic surfactant, ethanolated alkyl guanidine-amine complex.

Arquad S, C.S.=Arquad S cationic surfactant, n-alkyl trimethylammonium chlorides.

Comparison A=Chromated magnesium powder.

| Tradename:                  | Type of compound                                                     |
|-----------------------------|----------------------------------------------------------------------|
| Michelene 10                | Diamine fatty acid condensate.                                       |
| Michelene 15                | Do.                                                                  |
| Michelene 30                | Amine fatty acid condensate.                                         |
| Michelene 45                | Do.                                                                  |
| Michelene D-4               | Sulfated fatty acid amide.                                           |
| Muslor K                    | Blend of fatty acid esters and polyglycols with complex amino bases. |
| Onamine RO                  | High-molecular weight tertiary amine.                                |
| Onyx-ol 12                  | Mixed fatty acid monoethanolamine condensate.                        |
| Onyx-ol 336                 | Lauric acid diethanolamine condensate.                               |
| Sapamine PA                 | Carboxylic acid amide derivative.                                    |
| Solar NP liquid concentrate | Ethoxylated nonyl phenol.                                            |
| Unicote                     | Fatty nitrogen complex.                                              |
| Uniwax                      | Fatty amide complex.                                                 |
| Wilimid T                   | Polyalkylene amine.                                                  |

The invention having been thus described, other modifications will be obvious to those skilled in the art, and the scope of the invention is to be considered limited only by the scope of the appended claims.

I claim:

1. In a method for providing a corrosion resistant coating on particulate magnesium metal which includes contacting said metal with a hot alkali metal dichromate solution, the improvement which comprises: washing the resulting chromated particulate magnesium metal with a dilute dispersion containing at least 0.05 percent by weight of a hydrophobic, water-dispersable, oxygen-containing surface active agent, said agent having at least one uninterrupted carbon to carbon chain, said chain containing from 8 to 26 carbon atoms, and said agent containing at least one carbon oxygen polar group linkage, said linkage having sufficient polarity to provide an affinity for the chromated surface of said chromated magnesium.

2. In a method for providing a corrosion resistant coating on particulate magnesium metal which includes contacting said metal with a hot alkali metal dichromate solu-

tion, the improvement which comprises: washing the resulting chromated particulate magnesium metal with a dilute dispersion containing from 0.05 to 0.5 percent by weight of a hydrophobic, water-dispersable, oxygen-containing surface active agent, said agent having at least one uninterrupted carbon to carbon chain, said chain containing from 8 to 26 carbon atoms, and said agent containing at least one carbon oxygen polar group linkage, said linkage having sufficient polarity to provide an affinity for the chromated surface of said chromated magnesium; and drying the so-washed chromated particulate magnesium metal.

3. In a method for providing a corrosion resistant coating on particulate magnesium metal which includes contacting said metal with a hot alkali metal dichromate solution, the improvement which comprises: washing the resulting chromated magnesium metal with a dilute dispersion containing from 0.05 to 0.5 percent by weight of an acid salt of a long chain fatty acid amide having as substituents on said long chain at least two amine groups.

4. In a method for providing a corrosion resistant coating on particulate magnesium metal which includes contacting said metal with a hot alkali metal dichromate solution, the improvement which comprises: washing the resulting chromated magnesium metal with a dilute dispersion containing from 0.05 to 0.5 percent by weight of an ethanolated alkyl guanidine-amine complex.

#### References Cited by the Examiner

##### UNITED STATES PATENTS

|           |       |                |             |
|-----------|-------|----------------|-------------|
| 2,229,236 | 1/46  | Beck et al.    | 148—6.27 XR |
| 2,279,252 | 4/42  | Slunder        | 148—6.27 XR |
| 2,454,799 | 11/48 | Hart et al.    | 148—6.27 XR |
| 2,796,369 | 6/57  | Chester et al. | 148—6.2     |
| 2,887,418 | 5/59  | Whitby         | 148—6.2     |
| 2,894,864 | 7/59  | Ek et al.      | 148—6.27 XR |
| 2,918,390 | 12/59 | Brown          | 148—6.2     |
| 2,927,046 | 3/60  | Andrade        | 148—6.2 XR  |
| 2,974,029 | 3/61  | Comyn          | 148—6.2 XR  |
| 3,016,339 | 1/62  | Riou et al.    | 148—6.27 XR |
| 3,021,228 | 2/62  | Gibson et al.  | 148—6.2     |

RICHARD D. NEVIUS, Primary Examiner.

45 RAY K. WINDHAM, Examiner.